

Dec. 22, 1931.

C. S. JOHNSTON

1,837,969

RAILWAY CAR

Filed Oct. 27, 1927.

3 Sheets-Sheet 1



Inventor  
Charles S. Johnston  
By  
Oscar Hochberg,  
his Attorney.

Dec. 22, 1931.

C. S. JOHNSTON

1,837,969

RAILWAY CAR

Filed Oct. 27, 1927

3 Sheets-Sheet 2



Inventor  
Charles S. Johnston  
By  
Oscar Hochberg  
his Attorney

Dec. 22, 1931.

C. S. JOHNSTON

1,837,969

RAILWAY CAR

Filed Oct. 27, 1927

3 Sheets-Sheet 3



Inventor  
Charles S. Johnston

Oscar Hochberg,  
his Attorney

## UNITED STATES PATENT OFFICE

CHARLES S. JOHNSTON, OF GLENCOE, ILLINOIS, ASSIGNOR TO UNION METAL PRODUCTS COMPANY, OF CHICAGO, ILLINOIS, A CORPORATION OF DELAWARE

## RAILWAY CAR

Application filed October 27, 1927. Serial No. 229,169.

My invention relates to means for preventing or retarding the corrosion of certain of the walls of steel railway cars exposed to the chemical action of fumes, moisture and other deleterious agencies.

That portion of the metal wall sheathing adjacent the joint between the wall plates and supporting frame of a railway car is invariably the first to be affected by the corrosive action of any moisture confined in the joint.

The corrosion manifests itself initially in the form of discolored patches localized in the area immediately adjacent the joint, developing thin scale which finally becomes loosened and falls away, revealing another layer of oxide beneath and which in turn is exposed to the action of the moisture. Repeated scaling down of the plates results ultimately in the failure of the joint-adjacent area of the wall sheathing.

Such rapid oxidation and reduction of the wall sheathing in the area adjacent the joint at the floor portion of the car and the relatively slow destruction of the wall sheathing above the affected region, necessitates either the removal of the several panels making up the sheathing of the car for the purpose of cutting away the disintegrated lower portions thereof to permit the splicing of new plates to replace the damaged sections, or the cutting away of the worn sections from the remainder of the respective panel sections without removing the panels from the car.

The methods noted present two objectionable alternatives, the one involving the virtual dismantlement of the car with its attendant prohibitive cost and the other the impairment of the superstructure framing member; in the first case the rivets or welds holding the sheathing plates to the posts and the posts to the top and bottom framing longitudinal must be cut away to permit removal of the sheathing panels, and in the latter case the use of the cutting torch will seriously disturb the integrity of the posts during the cutting operation, since the heat of the cutting frame if not the flame itself, will penetrate the posts at the splice position, with resultant weakening of the posts, necessitating replacement or repair.

It is therefore the principal object of the invention to overcome the objections above outlined by forming the wall portion in the area adjacent the floor of the car of metal plate resistant to oxidation and to initially splice said plate to wall sheathing made up of plates lacking such property or affording relatively lower resistance to corrosion, to the end that the necessity for the renewal or repair of the wall plates may be minimized.

The foregoing and other objects are attained by the construction illustrated in the accompanying drawings, in which:

Fig. 1 is a side elevational view of a metal sheathed railway box car embodying the invention;

Fig. 2 is a vertical section taken at the longitudinal central line of the car showing the application of the invention to an end wall of the car;

Fig. 3 is a transverse vertical section taken at center of the body bolster of the car on line 3-3 of Fig. 1, looking in the direction indicated by the arrows, showing a preferred embodiment of the invention as applied to a box car;

Fig. 4 is a similar though fragmentary view of the splice plate arrangement on an enlarged scale;

Fig. 5 is a fragmentary view transversely of a car showing a modified construction embodying the invention;

Fig. 6 is a similar view showing the application of the invention to a box car having exterior framing members;

Fig. 7 is a side elevational view of a drop bottom gondola car embodying the invention; and

Fig. 8 is a transverse vertical section taken on line 8-8 of Fig. 7, looking in the direction indicated by the arrows, showing the application of the invention to gondola cars of this type.

In the drawings, 10 represents the side wall sheathing of a steel box or other house car secured to framing posts 11 terminating at and secured to framing longitudinal plates 12 and sills 13; and 14 indicates similar sheathing forming the end wall of the car and secured to end posts 15 connecting the

end plates (not shown) and end sills 16, shown in Fig. 2 of the drawings.

In the practice of the invention it is contemplated that the side and/or end wall 5 sheathing 10 and 14, respectively, will be made up of metal panels extending from the top plates to within a predetermined point above the floor 17 of the car, leaving an opening extending from the lower margin of the 10 respective sheathing plates to the side or end sills 13 and 16 and from post to post at the sides and ends of the car, the openings thus formed being closed in a manner presently to be described. The sheathing plates 10 and 15 14 terminate at a point above which the liberated corrosive acids present in or generated by the lading carried in the car are not expected to seriously curtail the useful life of the plates; thus positioned the plates are practically 20 free from direct attack by the chemical action of water and acid concentrations in the joints adjacent the floor line and would last indefinitely. Such plates may be made of a metal affording little or no resistance to 25 corrosion, depending upon the type of car and the predominant character of the lading to be carried.

The respective lower margins 18 of the 30 side and end wall plates 10 and 14 and contiguous areas of the plates are protected from the ravages of sulphuric acid from coal or acid waters from other lading, by means of intervening foot plates 20 of metal having a relatively high resistance to oxidation, or 35 coated with metal possessing that property; these plates extend downwardly from the lower margins 18 of side and end wall plates 10 and 14 to the respective side and end sills 13 and 16, and provide a wall area capable of 40 preventing or retarding the corrosive action of moisture in the joint 9 between said plates and sills. As shown in Fig. 1, the incorrodible or slow corroding foot plates 20 are arranged in lengths greater than the distance 45 between adjacent posts and preferably extending continuously between the corner posts 19 and door posts at the car sides and between said corner posts at the ends of the car to facilitate assembling and to provide a unitary 50 gusset connection between the posts and respective side and end sills and sheathing plates. The foot plates 20 at their upper edges overlap the lower margins 18 on the inner sides of the respectively adjacent wall 55 sheathing plates 10 and 14 and are preferably offset as indicated at 21 in Figs. 3, 4, and 6, to provide a watershed and a flush outer face at the joint 22, at once preventing the entrance of water to the car interior and substantially 60 reinforcing the car wall at the floor line.

As indicated in Fig. 6 of the drawings the invention may be adapted to house cars having exterior framing members 25 secured to outer faces of wall sheathing plates 10 and

foot plates 20, the flush joint 22 permitting the use of framing members without the necessity of offsetting them at that point. The framing members 25 are shown in this figure as commercial rolled Z-bars connected by 70 rivets 23 to wall sheathing plates 10, foot plates 20, and adjacent side sill 13; to insure proper bearing for the lower ends of said framing members below the respective foot plates 20, filler plates 24 are inserted between 75 the several framing members 25 and the side sill 13 and held by the rivets 23. In the embodiment shown the wall plates 10 are secured to the framing members 25 by vertical flanges 26 projecting outwardly from the base of the respective plates and lapping the webs 27 of the members, though obviously the wall plates 10 may overlap each other in the plane of the wall as indicated in Fig. 1 with the framing members 25 secured to the outer faces of the respectively adjacent plates. As in the case of the other embodiments the foot plates 20 lap under the relatively higher wall plates 10 to provide the watershed hereinbefore referred to, and are secured thereto by welding or riveting, as desired, and to the side sill 13 as shown in this figure.

Although the invention has been described with particular reference to box and other house cars, its usefulness is indicated in open top cars of the fixed bottom gondola type and hopper or other drop bottom cars. Such cars are peculiarly susceptible to corrosion because of the exposure of the cars and their lading to the elements; the effect of moisture and air upon the lading in producing acid waters and the pressure and erosive action of ore, rock, coal, etc., comprising a large proportion of the lading carried in such cars, are contributing factors in causing the rapid disintegration of the bottom load confining plates. Because of the unfavorable position of the plates most exposed to the corrosive action of agencies operating below the surface of the lading and near the bottom of the car, such plates soon become worn and must frequently be replaced before the plates in the upper areas of the car walls show any indication of corrosion. To that situation the present invention is directed; the plates, 100 most exposed to attack by the chemical action of air and moisture at or near the bottom of the car are made of metal having relatively greater resistance to oxidation than the plates constituting the upper areas of 105 the car walls.

In the embodiment illustrated in Figs. 7 and 8, a general service or drop bottom gondola car is shown equipped in accordance with the invention; the load deflecting plates 30 and diaphragm cover plates 31, are made from metal either immune or highly resistant to corrosion, and the upper wall plates 32 of metal having relatively little or no resistance to oxidation. This distribution 110

of plates having relatively different characteristics, coupled with the initial splicing of such plates, materially reduces the cost of maintenance, since the necessity for replacement of the plates will have been materially reduced.

The upper wall portions of the house and open top steel cars above noted may be of standard open-hearth process steel containing carbon not exceeding 0.18 percent, sulfur and phosphorous not in excess of 0.06 percent, respectively, and manganese not over 0.80 percent. Steel of this composition offers a relatively low resistance to corrosion. For the foot plates 20 of house and fixed bottom gondola cars, and shedding and cover plate portions 30 and 31, respectively of the drop bottom open top cars, steel plates of relatively high resistance to corrosion may be made by the addition of about 0.20 percent copper to the composition stated for the upper wall plates.

The character of some of the lading carried may warrant the use of non-corrodible or slow corroding plates in the upper wall areas of the cars, but whatever the resistance value of the metal in such upper wall plates, the lower wall areas are to be formed of metal affording a relatively higher resistance to corrosion, thereby insuring a longer life to the plates making up the lower wall portions of the car.

Within the scope of the invention, the use of metal plates is contemplated upon which has been sprayed, or deposited electrolytically, a thin coating of another metal to protect the underlying plate from acid corrosion. Should plates of very high resistance to corrosion be desired, such plates of chrome, vanadium, or other alloy steels having the relatively different characteristics hereinabove outlined may be substituted.

It should be noted that the underframe 8, including the side and end sill framing members 13 and 16 of the house car and the longitudinal member 33 of the open top car shown in Figs. 7 and 8 of the drawings, because of the heavier nature of the materials entering into its construction at respective joints 9, 50 may be of metal having corrosion resisting values not exceeding that required for the upper wall plates 10, 14, and 32, and relatively lower than contiguous plates 20 and 30 respectively of the house and open top cars.

What I claim is:—

1. A railway car having an underframe, and side and end wall plates arranged in connected upper and lower series, said upper series of plates having a lower resistance to oxidation than the lower series.

2. A railway car having an underframe, and side and end wall plates arranged in connected upper and lower series above the underframe, the surfaces of said upper se-

ries of plates having a lower resistance to oxidation than said lower series.

3. A railway car having an underframe, and side and end wall plates arranged in connected upper and lower series above the underframe, the plates comprising said upper wall courses having a lower resistance to oxidation than said lower series.

4. A railway car having an underframe, and side and end wall plates arranged in connected upper and lower series, said lower series of plates having a higher resistance to corrosion than the other series and the underframe.

5. A railway car having an underframe, and side and end walls comprising an upper series of plates having a relatively low resistance to corrosion, and a lower series of plates connecting said upper wall portions and the underframe and providing a relatively high resistance to oxidation.

6. A railway car having side and end walls and an underframe, the underframe and contiguous wall areas having relatively different resistance to corrosion.

7. A railway car having upper framing members and an underframe, and side and end wall plates connecting said underframe and framing members, said wall plates having areas of relatively high resistance to corrosion adjacent said underframe.

8. A railway car having an underframe, a series of side and end wall plates terminating with their lower margins at a predetermined point above the underframe, and wall plates of metal having a relatively high resistance to oxidation connecting said first mentioned wall plates and underframe.

9. A railway car having upper framing members and an underframe, a series of wall plates of metal having a relatively high resistance to oxidation secured to the underframe and framing, and an overlapping series of plates lacking such properties spliced to said first mentioned plates and secured to said framing.

10. In a railway car comprising an underframe and upper framing members, a series of wall plates secured to said upper framing and terminating with their lower edges at a predetermined point above the underframe, and incorrodible or slow corroding reinforcing gusset plates secured to the underframe and secured along their upper margins to contiguous edges of the other wall plates to provide a weather-proof joint.

11. In a railway car having an underframe and a series of wall sheathing plates having their lower marginal edges spaced above the underframe, and a plurality of foot-plates connecting said underframe and sheathing plates and secured along their upper edges to contiguous edges of a plurality of the sheathing plates, said foot-plates providing

- areas having a relatively high resistance to oxidation.
12. In a railway car having an underframe and an upper series of wall sheathing plates having their lower marginal edges terminating at predetermined points above the underframe, and gusset plates severally connecting a plurality of said sheathing plates and underframe and providing areas having a higher resistance to corrosion than the other plates and said underframe.
13. A railway car having an underframe, an upper series of wall plates with their lower edges terminating at predetermined points above the floor line of the car, and a lower series of plates having a relatively high resistance to oxidation connecting said upper plates to the underframe.
14. In a railway car having side and end walls and an underframe, an upper series of wall plates having little or no resistance to corrosion, and a lower series of wall plates relatively immune to corrosion connecting said upper wall plates to the underframe, said lower series of plates being spliced to the other plates.
15. In a railway car, a girder forming a wall of the car, said girder comprising a top rolled metallic chord, a bottom rolled metallic chord, a rolled metallic plate forming the upper part of the web of the girder, and a cast metal member forming the lower part of the web of the girder.
16. In a metal wall structure for cars having a top plate and sill, the combination with a sheet metal panel secured at its upper edge to the plate and having its lower edge terminating above said sill; of a casting extending along the bottom edge of the panel and secured thereto and extended to and secured to the sill to complete the wall.
17. In a metal wall structure for cars having a top plate and sill, the combination with a plurality of vertically extending sheet metal panels secured along their adjacent vertical edges, said panels being secured along their upper edges to the plate and terminating above the sill at their lower edges; of a plurality of castings extending along the bottom edges of the panels and secured thereto, said castings also being secured to the sill.
18. In a metal wall structure for cars, the combination with a side plate; of a side sill; vertically extending sheet metal panels having their upper edges secured to said side plate and terminating above the side sill; and horizontally elongated castings secured along their upper edges to the lower edges of the panels, said castings being secured along their bottom portions to the side sill.
19. As an article of manufacture, a casting for car wall structure, said casting being elongated and formed along its bottom portion to fit against and be secured to a sill, said casting having an upwardly extending web sec-
- tion adapted to be secured to a sheet metal panel.
20. In a railway car, a wall and a floor forming load retaining means thereof, the portion of the wall adjacent the floor being of relatively non-corrosive material and the portion of the wall remote from the floor being of relatively corrosive material.
21. In a railway car structure, the combination of a member forming the lower portion of a wall of said car which is composed of relatively non-corrosive material, and an element forming the upper portion of said wall which is composed of relatively corrosive material.
- In witness whereof I have hereto set my hand this 13th day of October, 1927.
- CHARLES S. JOHNSTON.

70

75

80

85

90

95

100

105

110

115

120

125

130